

Aug. 2, 1960

G. M. MOELTER

2,947,595

TREATMENT OF FILAMENTARY MATERIALS

Filed Jan. 24, 1955



INVENTOR.

GREGORY M. MOELTER

BY

*G. M. Moelter*  
ATTORNEYS

1

2,947,595

## TREATMENT OF FILAMENTARY MATERIALS

Gregory M. Moelter, Bernardsville, N.J., assignor to Celanese Corporation of America, New York, N.Y., a corporation of Delaware

Filed Jan. 24, 1955, Ser. No. 483,601

16 Claims. (Cl. 8—151.2)

This invention relates to the treatment of filamentary materials and relates more particularly to the continuous treatment of filamentary materials with liquids.

It is common in the art to treat filamentary materials with liquids in a continuous manner. For example, one treatment of this type which has come into wide use involves the continuous desulfurizing, washing and bleaching, without intermediate winding operations, of freshly spun continuous filaments of viscose rayon. For such continuous treatments, machines known as thread-storage thread-advancing devices are employed. Generally, these are driven reel-like structures around which the filamentary material is caused to pass continuously in a helical path while it is subjected to the treatment with the liquid or liquids. Such devices are not entirely satisfactory since they are usually bulky, expensive, complicated, difficult to string up, and prone to cause breaks in the filaments, resulting in entanglement of the filaments and in shutdown of the devices.

It is therefore one object of this invention to provide a novel process for the continuous treatment of filamentary materials with liquids, and a novel thread-storage, thread-advancing device for carrying out such treatment, which will be free from the foregoing and other difficulties.

Another object of this invention is the provision of a new and improved method and apparatus for the continuous liquid treatment of filamentary materials in an efficient and economical manner.

Other objects of this invention will be apparent from the following detailed description and claims.

In accordance with one aspect of this invention the filamentary material to be treated is introduced into a bath of treating liquid continuously in the form of a series of closed, or crunodal, loops arranged in a spiral whose diameter is greater than the diameter of said loops. Successive convolutions of this spiral rest on one another so that an annular mass of the filamentary material is built up in the treating bath. The treated filamentary material is withdrawn continuously, in uncoiled form, from the bottom of this mass of filamentary material.

In one convenient form of apparatus for carrying out this invention, the filamentary material and the treating liquid are fed continuously to a funnel to form a stream which falls freely from the funnel to the bath of treating liquid. The lower end of the funnel is moved continuously in a substantially circular path about a vertical axis so that a spiral motion is imparted to the falling stream of liquid and yarn. The bath of treating liquid is contained in a U-tube having an entrance arm and an exit arm. The entrance arm of the U-tube is constricted at a point below the surface of the bath. This constriction serves to support the spiral mass of filamentary material which forms in said entrance arm. The treated yarn is withdrawn in uncoiled condition and under some tension from the bottom of this spiral mass and up through the exit arm of said U-tube.

2

It is desirable that the diameter of the spiral of yarn be somewhat smaller than the internal diameter of the entrance arm of the U-tube. For example, for a U-tube of 1 1/4 inch internal diameter, a suitable spiral has a diameter of about 3/4 inch. This permits the coils of the spiral to move downwardly freely in the treating liquid but prevents the spiral from toppling over and becoming entangled.

While best results have thus far been attained by the use of a U-tube it will be understood that other means for containing the bath of treating liquid and for supporting the spiral mass of filamentary material may be employed. For example, a straight tube constricted at its lower end may be supported in a relatively large tank filled with treating liquid and the filamentary material may be spiraled into this straight tube and withdrawn under some tension from the bottom of the tube and through the tank. Such a tube may be perforated or slotted, if desired. In fact, the straight tube may be replaced entirely by suitable spaced guide members, for example, by parallel circularly disposed guide bars converging at their lower ends, which guide bars serve to keep the spiral mass of filamentary material in place. Also, although it is most advantageous that the filamentary material be formed into a generally circular spiral and the treatment tube be of generally circular cross-section, shapes other than circular, e.g. elliptical or oval, may be employed, if desired. It is preferred that the spiral mass of filamentary material be disposed substantially vertically during the process. However, if desired, the tubes or guide members may be so arranged that this spiral mass is disposed at an angle to the vertical, e.g. an angle of 30° to the vertical.

It is generally advantageous to combine the filamentary material with a stream of liquid before the filamentary material enters the treating bath. The liquid stream adds weight to the yarn so that it feeds more freely into the bath. However, if desired, the yarn may be introduced into the treating bath without first coming into contact with the liquid, or the yarn may be merely moistened with the liquid before it enters the treating bath. The liquid may then be fed to the treating bath at some other point. Thus, a stream of treating liquid may be introduced into the exit arm of the U-tube and the liquid may be removed continuously from the entrance arm, so that the liquid and yarn move in opposite directions and there is a countercurrent treatment of the yarn.

If desired, a moving, rather than a stationary, treating bath may be employed while the yarn falls into the moving bath from a stationary, rather than a moving point. Thus, the U-tube holding the treating bath may be moved as a unit about a vertical axis, e.g. in a circular path about an axis parallel to the path of the falling yarn, or the U-tube may be pivoted at the bottom and the top of the U-tube, and the surface of the bath, moved in a closed path about such a vertical axis.

It will be understood, of course, that a series of treating liquids may be applied to the filamentary material by the process of this invention. Thus, a yarn may be passed first through an apparatus of the type described containing a liquid reactive with said filamentary material and then directly without intermediate winding through one or more similar pieces of apparatus containing other reactive liquids or washing liquids.

The process of this invention may be carried out using any desired filamentary material and any desired treating liquids. For example, it may be employed for the successive acetylation and washing of incompletely acetylated cellulose acetate yarns; for the desulfurizing and washing of freshly coagulated regenerated cellulose yarns made from viscose, or for the saponification of cellulose acetate

filaments. The filamentary material may be in the form of yarn of high or low denier or it may be in the form of a tow of, for example, 100,000 or 200,000 denier containing many thousands of individual filaments, if desired. However, this invention shows its greatest practical benefit for yarns of less than about 25,000 denier rather than heavy tows, since the ordinary handling and treating of such tows does not present as great a problem of tangling as the handling and treatment of yarns.

By the use of the process and apparatus of this invention the filamentary material is treated efficiently and economically in a continuous manner without developing tangles, snarls, slubs or broken filaments.

The accompanying drawing illustrates one form of the apparatus of this invention wherein,

Fig. 1 is a diagrammatic side view of the apparatus of this invention, with parts thereof in cross section,

Fig. 2 is an enlarged cross sectional side view of a portion of the apparatus shown in Fig. 1, and

Fig. 3 is a plan view, taken along the line 3—3 of Fig. 2, showing the general appearance of the upper convolution of the spiral mass of filamentary material.

Like reference numerals indicate like parts throughout the several views of the drawing.

Referring now to the drawing, reference numeral 11 indicates a yarn, composed of a number of continuous filaments, which may be twisted or untwisted as desired. The yarn 11 is fed positively and continuously from a suitable source of supply, not shown, by a pair of driven feed rolls 12 into the large conical portion 13 of a funnel 14. A treating liquid from a supply hereinafter referred to is fed to the funnel 14 through a pipe 16 having a valve 17. The yarn 11 and the liquid leave the funnel 14 together through the stem 18.

The apparatus is constructed and arranged to impart a spiral motion to the stream of liquid and yarn leaving the lower end of the stem 18 of the funnel 14. To this end the funnel 14 is loosely supported by, and passes through, an apertured plate 19, with the upper edge of the aperture 21 in said plate engaging the conical portion 13 of the funnel near the point where said conical portion joins the stem 18. The aperture 21 is of larger diameter than the stem 18. Any suitable mechanical device, such as the arrangement of the motor 22 and slidably mounted eccentric member 23 illustrated diagrammatically in drawing Fig. 1, serves to move the bottom portion of the stem 18 in a substantially circular path about a vertical axis, such circular motion being permitted by the loose connection between the funnel 14 and the apertured plate 19.

The spiralling stream of treating liquid and yarn falls freely from the funnel into arm 24, hereinafter referred to as the entrance arm, of a U-tube 26 partly filled with said treating liquid, which is maintained at the desired predetermined level by means of a flexible and adjustable overflow device 27, of conventional construction, attached to the second arm 28, hereinafter referred to as the exit arm, of said U-tube. As the yarn passes into the liquid in the entrance arm 24, it takes the form of a series of small closed, or crunodal, loops arranged in a spiral whose diameter is greater than the diameter of said loops. As shown in Fig. 3, each coil of this spiral of yarn 11 has the general appearance of a prolate epitrochoid, which is the curve described by a point on the prolongation of the radius of a circle as said circle rolls along the outside of a fixed circle.

The entrance arm 24 of the U-tube 26 is constricted at a point spaced below the level of the liquid therein, as by a plurality of circumferentially spaced hemispherical portions 29 projecting into the interior of said arm. The yarn, being of higher density than the liquid, settles in the arm 24 until it rests on the inwardly projecting portions 29 and builds up, with each successive coil of the spiral of yarn resting on the preceding coil, to form a generally cylindrical annular mass 31. When this mass of

yarn has built up to the desired level, which is generally the same as the level of the liquid in the arm or slightly higher, e.g.  $\frac{1}{2}$  inch higher, the lowest portion of the yarn 11 is withdrawn continuously past the inwardly projecting portions 29 and out of the exit arm 28, around a stripping guide 32, which serves to remove liquid from the yarn, through a traversing guide 33 of the usual type, and onto a driven rotating bobbin 34 or other suitable support where it is wound in the form of a package. The rate at which the yarn is withdrawn by the action of the bobbin 34 is so related to the rate at which the yarn is fed by the rolls 12 that substantially steady-state conditions are maintained in the U-tube 26. That is, if the treatment is such that the yarn does not change in length during the treatment, the linear rate of withdrawal is substantially equal to the rate of feed, while if the yarn increases or decreases in length during the treatment the linear rate of withdrawal is proportionately higher or lower, respectively, than the rate of feed.

It will be understood of course that in starting the treating operation it will be convenient first to pass the yarn through the entire U-tube 26, then to feed the yarn into the entrance arm 24 without withdrawing any yarn from the U-tube and then, when the mass 31 of yarn in the entrance arm 24 has built up to the desired level, to begin the withdrawal of the yarn from the exit arm 28.

Under some conditions there is a tendency for the mass 31 of yarn supported above the inwardly projecting portions 29 to become packed against the inner walls 30 of the entrance arm 24 of the U-tube and to impede the free movement of treating liquid around the outside of said mass of yarn. To overcome this tendency the entrance arm 24 is so constructed as to provide one or more passageways or channels for such free flow of liquid. As shown in Fig. 3 the interior of the entrance arm 24 is fluted for this purpose.

In order to maintain the treating liquid at the desired predetermined temperature the U-tube 26 may be insulated or fitted with a heating or cooling jacket 36.

The treating liquid overflowing from the U-tube 26 is led from the overflow device 27, past a valve 39, to a storage reservoir 41 from which it is withdrawn and recirculated to the feed pipe 16 by means of a pump 42. If desired, the reservoir 41 may be by-passed and the liquid recycled directly through a pipe 43 and valve 44 to the feed pipe 16.

It will be understood that the time of treatment, i.e. the residence time of the filamentary material in the treating liquid, may be regulated by appropriate changes in the amount of material in the spiral mass 31. This may be done, for example, by temporarily speeding up or slowing down the rate of withdrawal of the filamentary material or the rate of feed of such material until the spiral mass 31 is of the desired size and then resuming the original rates of withdrawal or feed. The time of treatment may also be changed by raising or lowering the level of the treating liquid in the U-tube by suitable adjustment of the overflow device 27. In addition, the time of treatment may be regulated, while keeping the size of the spiral mass 31 constant, by appropriate changes in both the feed rate and the withdrawal rate. Combinations of all these methods may be employed, if desired.

The following example is given to illustrate this invention further. All proportions are by weight unless otherwise indicated.

#### Example

The apparatus described above is employed for the continuous acetylation of a 2000 denier untwisted yarn composed of 1350 filaments of stretched, oriented cellulose acetate having an acetyl value of 54.3%, calculated as combined acetic acid. The yarn is fed at a constant speed of 75 meters per minute into the funnel, whose upper conical portion is tapered at an angle of  $60^\circ$  (included angle) and whose stem is 2 inches in length and  $\frac{1}{8}$  inch

in internal diameter. An acetylation mixture of 8.3% of acetic anhydride, 0.5% of acetic acid, 0.2% of sulfuric acid and 91.0% of benzene, at a temperature of 60° C., is fed into the funnel at a constant rate of 0.50 liter per minute. The bottom of the stem of the funnel is rotated, about a vertical axis, at a rate of 60 r.p.m. in a circle  $\frac{1}{2}$  inch in diameter. The yarn and acetylation mixture fall freely from the stem to the entrance arm of the U-tube, which U-tube has an internal diameter of  $\frac{1}{4}$  inches and an overall height of 35 inches. The arms of the U-tube are vertical and of equal height, their center lines are spaced  $\frac{5}{8}$  inches apart and the exit arm of the U-tube is provided with a device for maintaining the level therein 15 inches from the tops of said arms. The inwardly projecting portions of the entrance arm have radii of  $\frac{3}{16}$  inch and are situated 25 inches from the top of the entrance arm, which is itself 13 inches below the bottom of the funnel. The yarn plait into entrance arm in the form of a series of crunodal loops about  $\frac{1}{4}$  inch in diameter, substantially symmetrically arranged about the center of the entrance arm, to form an annular pattern about  $\frac{3}{4}$  inches in diameter. When this annular pattern has been built up to the level of the treating liquid in the U-tube, i.e. to a height of 10 inches above the inwardly projecting portions in the entrance arm, the yarn is withdrawn from the exit arm of the U-tube at such a rate that steady state conditions are maintained. Under these conditions the residence time of the yarn in the tube is 3 minutes and the yarn leaving the tube has an acetyl value of over 61%. The apparatus operates continuously for long periods of time without developing tangles, snarls, slubs or broken filaments in the yarn.

It is to be understood that the foregoing detailed description is given merely by way of illustration and that many variations may be made therein without departing from the spirit of my invention.

Having described my invention what I desire to secure by Letters Patent is:

1. In the process for the liquid treatment of filamentary material, the individual filaments of which all extend substantially in the direction of the length of said filamentary material, the improvement which comprises introducing said filamentary material into a liquid treating bath continuously in the form of a series of crunodal loops of said filamentary material arranged in a spiral having a diameter greater than the diameter of said loops, supporting said spiral in said bath with successive convolutions of said spiral resting on one another, and continuously withdrawing said filamentary material from the bottom of said spiral.

2. In the process for the liquid treatment of filamentary material, the individual filaments of which all extend substantially in the direction of the length of said filamentary material, the improvement which comprises introducing said filamentary material into a liquid treating bath continuously in the form of a series of crunodal loops of said filamentary material arranged in a spiral having a diameter greater than the diameter of said loops, the density of said liquid bath being less than the density of said filamentary material whereby said spiral of yarn loops sinks in said bath, supporting said spiral in said bath with successive convolutions of said spiral resting on one another, and continuously withdrawing said filamentary material from the bottom of said spiral.

3. In a process for the liquid treatment of filamentary material, the individual filaments of which all extend substantially in the direction of the length of said filamentary material, the improvement which comprises introducing said filamentary material into a liquid treating bath continuously in the form of a series of crunodal loops of said filamentary material arranged in a substantially vertical, annular spiral having a diameter greater than the diameter of said loops, supporting said spiral in said bath with successive convolutions of said spiral resting

on one another, and continuously withdrawing said filamentary material from the bottom of said spiral.

4. In the process for the liquid treatment of filamentary material, the individual filaments of which all extend substantially in the direction of the length of said filamentary material, the improvement which comprises continuously introducing a treating liquid and said filamentary material into a liquid treating bath, contained in a U-tube, continuously in the form of a series of crunodal loops of said filamentary material arranged in one arm of said U-tube in the form of a substantially vertical annular spiral having a diameter greater than the diameter of said loops, said spiral being supported in said arm with successive convolutions of said spiral resting on one another, and continuously withdrawing the yarn from the bottom of said spiral in unlooped condition through said U-tube.

5. Process for the liquid treatment of filamentary material the individual filaments of which all extend substantially in the direction of the length of said filamentary material, which comprises continuously feeding said filamentary material, feeding a liquid for treating the same into contact with said filamentary material to form a continuous stream containing said liquid and filamentary material, passing said stream downward in free condition from a point while rotating said point about a horizontal axis, introducing said stream into a bath of said liquid, said liquid being of lower density than said filamentary material, said filamentary material introduced into said bath forming a series of crunodal loops arranged in a spiral having a diameter greater than the diameter of said loops, supporting and maintaining said spiral with successive convolutions of said spiral resting on one another, and continuously withdrawing said yarn from the bottom of said spiral in unlooped condition.

6. Apparatus for the liquid treatment of filamentary material, which comprises means for supplying a filamentary material the individual filaments of which all extend substantially in the direction of the length of said filamentary material, means for providing a bath of treating liquid, means for continuously introducing said filamentary material into said bath in the form of a series of crunodal loops arranged in a spiral having a diameter greater than the diameter of said loops, mean for supporting said spiral in said bath with successive convolutions of said spiral resting on one another, and means for continuously withdrawing said filamentary material from the base of said spiral in uncoiled condition, said introducing means comprising means for bringing together said filamentary material and said treating liquid to form a continuous stream and for introducing said stream from a point into said treating bath, and means for moving said point in a closed path about a substantially vertical axis to impart a spiral motion to said stream.

7. Apparatus for the liquid treatment of filamentary material, which comprises means for supplying a filamentary material the individual filaments of which all extend substantially in the direction of the length of said filamentary material, means for providing a bath of treating liquid and means for continuously introducing said filamentary material into said bath in the form of a series of crunodal loops arranged in a spiral having a diameter greater than the diameter of said loops, said introducing means comprising means for bringing together said filamentary material and said treating liquid to form a continuous stream and for introducing said stream from a point into said treating bath, and means for moving said point in a closed path about a substantially vertical axis to impart a spiral motion to said stream.

8. Apparatus for the liquid treatment of filamentary material, which comprises means for supplying a filamentary material the individual filaments of which all extend substantially in the direction of the length of said filamentary material, means for providing a bath of treating liquid and means for continuously introducing said filamentary material into said bath in the form of a series

of crunodal loops arranged in a spiral having a diameter greater than the diameter of said loops, said introducing means comprising a tube spaced above said bath, means for continuously feeding said filamentary material and said treating liquid to said tube to form a stream which falls to said bath, and means for moving the bottom portion of said tube in a closed path about a substantially vertical axis to impart a spiral motion to said falling stream.

9. Apparatus for the treatment of filamentary material, which comprises means for supplying a filamentary material the individual filaments of which all extend substantially in the direction of the length of said filamentary material, a U-tube adapted to be filled at least partly with a treating liquid, means for continuously introducing said filamentary material into said treating liquid in one arm of said U-tube in the form of a series of crunodal loops arranged in a spiral having a diameter greater than the diameter of said loops, means for supporting said spiral with successive coils of said spiral resting on one another, and means for continuously withdrawing said filamentary material from the bottom of said spiral through said U-tube in uncoiled condition, said introducing means comprising means for bringing together said filamentary material and said treating liquid to form a continuous stream and for introducing said stream from a point into said arm, and means for moving said point in a closed path about a substantially vertical vertical axis to impart a spiral motion to said stream.

10. Apparatus as set forth in claim 9, said supporting means comprising a constriction in said U-tube.

11. Apparatus as set forth in claim 9, said introducing means comprising a funnel, means for continuously feeding said filamentary material and said treating liquid to said funnel to form a stream which falls to said treating liquid in said arm and means for moving the bottom portion of said funnel substantially in the path of a circle, whose diameter is less than the diameter of said arm, about a substantially vertical axis to impart a spiral motion to said falling stream.

12. Apparatus as set forth in claim 11, said supporting means comprising projections extending inwardly from the walls of said arm of said U-tube, said walls being fluted to provide channels for the free movement of said liquid around said spiral, said withdrawing means being constructed and arranged to withdraw said filamentary material through the other arm of said U-tube, said apparatus also including overflow means for continuously removing said treating liquid from said other arm and for maintaining said liquid at a predetermined constant level in said U-tube.

13. Apparatus for the liquid treatment of filamentary material, which comprises means for supplying a filamentary material the individual filaments of which all extend substantially in the direction of the length of said filamentary material, means for providing a bath of treating liquid, means for continuously introducing said filamentary material into said bath in the form of a series of crunodal loops of said filamentary material arranged in a spiral having a diameter greater than the diameter of said loops, means for providing a passageway for the movement of said filamentary material in said bath and for supporting said spiral in said bath with successive convolutions of said spiral resting on one another, said passageway having a constriction preventing movement of said spiral mass therethrough, and means for withdrawing said filamentary material in uncoiled condition from said spiral mass through said constriction, said introducing means comprising means for bringing together said filamentary material and said treating liquid to form a continuous stream and for introducing said stream from a point into said treating bath, and means for moving said point in a closed path about a substantially vertical axis to impart a spiral motion to said stream.

14. Process which comprises continuously passing a yarn of less than about 25,000 denier together with a liquid for treating the same and in contact therewith into a liquid treating bath and in the form of a series of crunodal loops of said yarn arranged in a spiral having a diameter greater than the diameter of said loops, supporting said spiral in said bath and above the bottom of said bath with successive convolutions of said spiral resting on one another, and continuously withdrawing said filamentary material from the bottom of said spiral.

15. Process as set forth in claim 2 in which said filamentary material is a yarn of less than about 25,000 denier.

16. Apparatus as set forth in claim 7 in which said means for providing a bath of treating liquid comprises a stationary container for said bath.

References Cited in the file of this patent

UNITED STATES PATENTS

|           |                  |                |
|-----------|------------------|----------------|
| 971,778   | Palmer           | Oct. 4, 1910   |
| 1,062,245 | Mathesius et al. | May 20, 1913   |
| 1,074,568 | Gant             | Sept. 30, 1913 |
| 1,475,428 | Carter           | Nov. 27, 1923  |
| 1,557,830 | Gurley           | Oct. 20, 1925  |
| 2,355,071 | Hendrickson      | Aug. 8, 1944   |
| 2,404,742 | Polack et al.    | July 23, 1946  |
| 2,634,596 | Pendleton et al. | Apr. 14, 1953  |
| 2,720,443 | Kegin            | Oct. 11, 1955  |